# EUROPEAN PATENT SPECIFICATION

(11) **EP 3 378 973 B1**
(45) Date of publication and mention of the grant of the patent: **29.06.2022**
(21) Application number: 17162054.5
(22) Date of filing: 21.03.2017
(51) Int. Cl.: C25D 3/06, C25D 5/48, C25D 9/10

(54) **METHOD FOR MANUFACTURING CHROMIUM-CHROMIUM OXIDE COATED BLACKPLATE**
VERFAHREN ZUR HERSTELLUNG EINER CHROM-CHROMOXIDBESCHICHTETEN SCHWARZBLECH
PROCÉDÉ DE FABRICATION D'UNE TÔLE NOIRE REVÊTUE D'OXYDE CHROME ET CHROME

(43) Date of publication of application: 26.09.2018
(73) Proprietor: Tata Steel IJmuiden B.V., 1951 JZ Velsen-Noord (NL)
(72) Inventor: WIJENBERG, Jacques Hubert Olga Joseph, 1970 CA IJmuiden (NL); WITTEBROOD, Adrianus Jacobus, 1970 CA IJmuiden (NL)
(74) Representative: Group Intellectual Property Services

(56) References cited:
- WO-A1-2014/202316
- WO-A1-2015/177314
- JP-A- H11 200 091
- JP-A- 2016 060 918
- US-A- 4 167 460

## Description

This invention relates to a method for electroplating an uncoated steel strip with a plating layer and an improvement thereof.

In continuous steel strip plating, a cold-rolled steel strip is provided which is usually annealed after cold-rolling to soften the steel by recrystallisation annealing or recovery annealing. After the annealing and before plating the steel strip is first cleaned for removing oil and other surface contaminants. After the cleaning step, the steel strip is pickled in a sulphuric or hydrochloric acid solution for removing the oxide film. Between different treatment steps the steel strip is always rinsed with deionised water to prevent contamination of the solution used for the next treatment step with solution of the preceding treatment step. Consequently the steel strip is thoroughly rinsed after the pickling step. During rinsing and transport of the steel strip to the plating section a fresh thin oxide layer is formed instantly on the bare steel surface and needs to be protected quickly.

One such process used in electroplating is called electrodeposition. The part to be plated (the steel strip) is the cathode of the circuit. The anode of the circuit may be made of the metal to be plated on the part (dissolving anode, such as those used in conventional tinplating) or a dimensionally stable anode (which does not dissolve during plating). The anode and cathode are immersed in an electrolyte solution containing ions of the metal to be deposited onto the blackplate substrate.

Blackplate is a tin mill product which has not (yet) received any metallic coating during production. It is the basic material for the production of other tin mill products. Blackplate can be single reduced (SR) full-hard or annealed (recovery annealed or recrystallisation annealed) or double reduced (DR) in which case it has been subjected to a second cold rolling reduction after annealing. The SR or DR blackplate is usually provided in the form of a coiled strip and is the uncoated starting material for the coating process according to the invention. Figure 1 schematically summarises the process steps to obtain the coated product, starting from a hot-rolled strip. Before cold-rolling, the hot-rolled strip is usually pickled (not shown) to remove the hot-rolling scale and cleaned (not shown) to remove any contaminants from the strip.

In the production of packaging steels with an electroplated chromium coating from an electrolyte solution comprising a trivalent chromium compound on an uncoated steel strip (blackplate), as disclosed in WO2014202316-A1, it occurs occasionally that at lower line speeds, the resulting coated product has a stripy appearance. Although the stripes are very faint and cannot be detected with XPS and/or SEM, they are nevertheless visible with the naked eye. The pattern appears to be even more visible when a clear lacquer coating (thermosetting coating) or polymer coating (thermoplastic coating) is applied onto the coated product. Although the coated product performs just as well in terms of corrosion performance, coatability, adherence of the lacquer coating or polymer coating to the coated product and the can-making performance of the coated product, no adverse effects have been observed of the presence of the stripes, the stripy appearance is considered to be visually less appealing and therefore undesired.

It is the object of the invention to improve the surface appearance of an electroplated chromium coating from an electrolyte solution comprising a trivalent chromium compound on an uncoated (blackplate) steel strip.

The object is reached with a method for manufacturing a chromium metal - chromium oxide coated blackplate by electrolytically depositing the chromium metal - chromium oxide coating on blackplate in a continuous high speed plating line operating at a line speed of at least 50 m/min from an electrolyte solution comprising a trivalent chromium compound, wherein the electrolyte solution is free of chloride ions and free of a boric acid buffering agent, the electrically conductive substrate acts as a cathode and an anode comprising a catalytic coating of iridium oxide or a mixed metal oxide for reducing or eliminating the oxidation of Cr³⁺-ions to Cr⁶⁺-ions, wherein the electrolyte solution contains at most 250 mM Cr³⁺-ions, a complexing agent at a (complexing agent/Cr³⁺) molar ratio of at least 1:1 and at most 2.5:1, wherein the complexing agent is formate (HCOO⁻), 210 to 2800 mM of sodium sulphate (Na₂SO₄), a pH of between 1.5 and 3.0 measured at 25 °C, and wherein the plating temperature is between 30 and 70 °C.

Preferable embodiments are provided in the dependent claims. For the sake of clarity it is noted that 1 mM means 1 millimole/l.

Firstly, it is noted that the process, in an embodiment not according to the invention, is equally applicable to provide a chromium metal-chromium oxide coating on other metal substrates such as nickel plated steel strip.

Secondly, if the pH of the electrolyte solution becomes too high or too low, then sulphuric acid or sodium hydroxide may be added to adjust the pH to a value inside the desired range. Also different acids or bases may be used, but in view of the bath chemistry sulphuric acid and sodium hydroxide are preferable.

Thirdly, as blackplate any steel grade suitable for producing packaging steel may be used. By means of example, but not intended to be limited by this, reference is made to the steel grades for packaging applications in EN10202:2001.

A stripy appearance of a deposited surface is usually associated with a certain inhomogeneity in the electroplating process. A local difference in coverage or local differences in the composition of the coating layer may be the cause of the stripy appearance. It would be obvious to the skilled person to attempt to solve this problem by increasing the amount of deposited material by either increasing the amount of metal ions in the electrolyte, or by increasing the current density. WO2014202316-A1 discloses a Cr³⁺ electrolyte using 120 g/l (= 385 mM) basic chromium(III)sulphate. This resulted in the aforementioned stripy surface under some conditions, such as a low line speed. Surprisingly, the inventors found that by increasing the chromium(III) content in the electrolyte, the appearance of the coated strip worsened, and that the stripy appearance persisted. Surprisingly and counter-intuitively the inventors found that decreasing the amount of metal ions in the electrolyte resulted in a decrease in the stripy surface and that the surface becomes even and shiny when the coating was deposited in accordance with the process of the invention.

WO2014202314-A1 discloses Cr3+ electrolytes comprising between 80 and 200 g/l of chromium(III) sulphate.

The reduction of the pH of the electrolyte also appeared to have a beneficial effect on the surface appearance of the coated product. This also is counter-intuitive, because a lower pH decreases the efficiency of this particular plating process. The higher the pH of the electrolyte, the lower the current density that is needed to deposit a certain amount of chromium. An increase of 2.7 to 2.85 already results in a considerable increase in current density required for a certain plating thickness (as expressed in mg/m²). This effect is independent of the line speed, although the magnitude of the current density required for a certain plating thickness increases with increasing line speed. So also at higher line speeds, a lower pH results in a less efficient plating process. And, reducing the pH has a positive effect on the appearance of the coated blackplate in that the stripy appearance is absent.

The effect of a lower chromium content in the electrolyte solution is shown in Figure 2. The lower the chromium content, the lower the current density needed for a certain plating thickness.

In a preferred embodiment the complexing agent is added to the electrolyte solution as sodium formate (HCOONa).

In an embodiment wherein the Cr³⁺-ions are provided by a water soluble chromium(III) salt and wherein the water soluble chromium(III) salt preferably is one or more of the following water soluble chromium(III) salts:
- basic chromium(III)sulphate
- chromium(III)formate
- chromium(III)oxalate
- chromium(III)acetate.

These salts have proven to work well in the electrolyte as claimed. The use of basic chromium(III)sulphate and/or chromium(III)formate is preferable from the point of view of keeping the bath chemistry as simple as possible. The addition of these compounds does not introduce additional ion-types to the electrolyte. The use of the chromium(III)oxalate and/or chromium(III)acetate instead of, or in addition to, chromium(III)formate may be desired if a different complexing agent is needed.

In an embodiment the electrolyte solution contains at most 225 mM of Cr³⁺-ions and/or at least 100 mM of Cr³⁺-ions, preferably at least 125 mM of Cr³⁺-ions. This preferred range provides good results.

In an embodiment the pH of the electrolyte solution is at most 2.8, preferably at most 2.6 or 2.4, more preferably at most 2.2. Although the lower pH results in a less efficient plating process, the surface quality is much improved in that it shows no stripes.

The formate/Cr³⁺ molar ratio is at most 2.5:1. The formate-ion is needed as a complexing agent and the ratio of at most 2.5:1 has proven to be sufficient in most cases. Preferably the molar ratio is at most 2.0:1, more preferably 1.75:1. Preferably the molar ratio is at least 1.1:1, more preferably 1.25:1.

In an embodiment the electrolyte solution contains at least 75 mM and/or at most 600 mM of sodium formate. When using only sodium formate as the addition of formate, and no chromium(III)formate as the water soluble chromium salt, then at least 75 mM should be added, preferably at least 100 mM and even more preferably 200 mM. The maximum is preferably at most 600 mM of sodium formate. If also chromium(III)formate is added to the electrolyte solution as the water soluble chromium salt then the formate added this way needs to be subtracted from the sodium formate additions as given herein above. For example, if 50 mM of formate is added as chromium(III)formate, then the values for sodium formate become at least 25 mM, preferably at least 50 mM and even more preferably 150 mM. The maximum is preferably at most 550 mM of sodium formate.

The electrolyte solution contains at least 210 mM and/or at most 845 mM of sodium sulphate.

In a preferred embodiment the plating temperature is at least 40 °C, preferably at least 50 °C, more preferably at least 55 °C.

In an embodiment the line speed of the plating line is at least 100 m/min, more preferably at least 200 m/min.

In an embodiment the coated blackplate is further coated on one or both sides by a film lamination step or a direct extrusion step, with an organic coating consisting of a thermoplastic single layer, or a thermoplastic multi-layer polymer, preferably wherein the thermoplastic polymer coating is a polymer coating system comprising one or more layers comprising thermoplastic resins such as polyesters or polyolefins, acrylic resins, polyamides, polyvinyl chloride, fluorocarbon resins, polycarbonates, styrene type resins, ABS resins, chlorinated polyethers, ionomers, urethane resins and functionalised polymers; and/or copolymers thereof; and or blends thereof.

The blackplate provided with a chromium metal - chromium oxide coating obtained by the process according to the invention has a shiny coating is shiny and shows no stripy appearance. In an aspect not according to the invention, the chromium metal - chromium oxide coated blackplate obtainable by the process according to the invention is used in a process to produce containers for packaging purposes.

### EXAM PLE

An electrolyte was prepared having a sodium formate concentration of 20 g/l (294 mM), a sodium sulphate concentration of 80 g/l (563 mM) and a pH of 2.6, 2.15 and 2.0, and a chromium concentration of 10 g/l (192 mM). The formate/Cr³⁺ ratio = 1.53. At each of these pH-values the appearance is not stripy, with the better appearance being obtained with the lower pH-values. Stripe free and shiny surfaces were obtained at line speeds of 100 and 200 m/min or higher.

In addition to the improvement of surface appearance by the reduction in pH there are additional advantages as a result of the lower Cr³⁺ in comparison to the prior art of WO2014202316-A1 (Cr³⁺ = 385 mM, pH 2.6). The higher current efficiency has already been mentioned and shown in Figure 2. In addition, because of the lower concentrations in the electrolyte, the degree of dragout losses will also be reduced. It is also believed that the edge build-up is reduced, and the lower sulphate content of the electrolyte is likely to result in lower sulphate contents in the deposited coating layer, which is beneficial for lacquer adherence.

The deposition mechanism of the chromium layer from the electrolyte solution according to the invention is assumed to be based on a fast, stepwise deprotonation of the water ligands in the Cr³⁺-formate complex ion induced by a surface pH increase as a result of hydrogen evolution (2H⁺ + 2e⁻ → H₂(g)) (See Figure 3 and 4):

[Cr(HCOO)(H₂O)₅]²⁺ + OH⁻ → [Cr(HCOO)(OH)(H₂O)₄]⁺ + H₂O (regime I)

[Cr(HCOO)(OH)(H₂O)₄]⁺ + OH⁻ → Cr(HCOO)(OH)₂(H₂O)₃↓ + H₂O (regime II)

Cr(HCOO)(OH)₂(H₂O)₃↓ + OH⁻ → [Cr(HCOO)(OH)₃(H₂O)₂]⁻ + H₂O (regime III)

In regime II (See Figure 4), a mixed Cr-metal-carbide-oxide coating is deposited on the steel substrate. In regime I there is no deposition of chromium, and in regime III the amount of deposited chromium drops sharply.

The current density at which the desired chromium coating weight and composition are obtained, depends on the electrolyte composition, pH, temperature and mass transfer rate (strip speed in case of a strip plating line). In practice, the optimal current density is not a discrete value, but a range of values restricted by a lower and an upper limit. This current density range is called the 'plating window'. Within the plating window, the coating properties fall within certain specifications. From an operational perspective, a large plating window is desired, because this simplifies process control.

Experiments (not according to the invention) were performed for investigating the influence of the chromium and formate concentration on the plating window.

**TABLE 1: RCE-EXPERIMENTS**

| electrolyte solution | I | | II | | III | |
|---|---|---|---|---|---|---|
| | g l⁻¹ | M | g l⁻¹ | M | g l⁻¹ | M |
| sulphate | 127.0 | 1.322 | 140.0 | 1.457 | 170.0 | 1.770 |
| TOC | 7.8 | 0.649 | 7.8 | 0.649 | 9.2 | 0.766 |
| Cr | 18.1 | 0.349 | 21.2 | 0.408 | 24.9 | 0.479 |
| Fe | 0.6 | 0.011 | 0.7 | 0.012 | 0.6 | 0.010 |
| Na | 49.8 | 2.164 | 58.0 | 2.523 | 61.1 | 2.658 |
| CrOHSO₄ basic chromium(III)sulphate | 57.6 | 0.349 | 67.3 | 0.408 | 79.0 | 0.479 |
| HCOONa sodium formate | 44.2 | 0.649 | 44.2 | 0.649 | 52.1 | 0.766 |
| Na₂SO₄ sodium sulphate | 107.6 | 0.758 | 133.1 | 0.937 | 134.4 | 0.946 |
| formate/Cr³⁺ molar ratio | 1.86 | | 1.59 | | 1.60 | |
| pH | 2.8 | | 2.8 | | 2.8 | |

| | | | | | | |
|---|---|---|---|---|---|---|
| TOC=Total Organic Carbon | | | | | | |

For the electrodeposition experiments titanium anodes comprising a catalytic coating or mixed metal oxide of iridium oxide and tantalum oxide are chosen. The rotational speed of the RCE was kept constant at 776 RPM (Ω^{0.7} = 6.0 s^{0.7}). The substrate was a 0.183 mm thick cold rolled blackplate material and the dimensions of the cylinder were 113.3 mm x ø 73 mm. The cylinders were cleaned and activated under the following conditions prior to plating.

**TABLE 2: PRETREATMENT OF THE SUBSTRATE**

| | step 1 | step 2 |
|---|---|---|
| | cleaning | activation |
| solution composition | 50 ml·l⁻¹ Chela Clean KC-25H | 25 g·l⁻¹ H₂SO₄ |
| temperature (°C) | 60 | 25 |
| current density (A·dm⁻²) | +1.5 (anodic) | 0 (dip) |
| Time (s) | 60 | 1.5 |

In figure 2 the results of coating trials with these compositions are given.

In a preferred embodiment an organic coating is provided on one or both sides of the chromium metal - chromium oxide coated blackplate substrate. It was found that organic coatings could be readily applied on to the chromium-chromium oxide coating, which itself acts a passivation layer to protect the electrically conductive substrate. The chromium-chromium oxide coating also exhibited good adhesion the subsequently applied organic coating. The organic coating may be provided as a lacquer or as a thermoplastic polymer coating. Preferably the thermoplastic polymer coating is a polymer coating system that comprises one or more layers of thermoplastic resins such as polyesters or polyolefins, but can also include acrylic resins, polyamides, polyvinyl chloride, fluorocarbon resins, polycarbonates, styrene type resins, ABS resins, chlorinated polyethers, ionomers, urethane resins and functionalised polymers. For clarification:
- Polyester is a polymer composed of dicarboxylic acid and glycol. Examples of suitable dicarboxylic acids include therephthalic acid, isophthalic acid, naphthalene dicarboxylic acid and cyclohexane dicarboxylic acid. Examples of suitable glycols include ethylene glycol, propane diol, butane diol, hexane diol, cyclohexane diol, cyclohexane dimethanol, neopentyl glycol etc. More than two kinds of dicarboxylic acid or glycol may be used together.
- Polyolefins include for example polymers or copolymers of ethylene, propylene, 1-butene, 1-pentene, 1-hexene or 1-octene.
- Acrylic resins include for example polymers or copolymers of acrylic acid, methacrylic acid, acrylic acid ester, methacrylic acid ester or acrylamide.
- Polyamide resins include for example so-called Nylon 6, Nylon 66, Nylon 46, Nylon 610 and Nylon 11.
- Polyvinyl chloride includes homopolymers and copolymers, for example with ethylene or vinyl acetate.
- Fluorocarbon resins include for example tetrafluorinated polyethylene, trifluorinated monochlorinated polyethylene, hexafluorinated ethylene-propylene resin, polyvinyl fluoride and polyvinylidene fluoride.
- Functionalised polymers for instance by maleic anhydride grafting, include for example modified polyethylenes, modified polypropylenes, modified ethylene acrylate copolymers and modified ethylene vinyl acetates.

Mixtures of two or more resins can be used. Further, the resin may be mixed with anti-oxidant, heat stabiliser, UV absorbent, plasticiser, pigment, nucleating agent, antistatic agent, release agent, anti-blocking agent, etc. The use of such thermoplastic polymer coating systems have shown to provide excellent performance in can-making and use of the can, such as shelf-life.

The application process of the thermoplastic polymer coating is preferably performed by laminating a polymer film onto the coated blackplate by means of extrusion coating and lamination, wherein a polymer resin is melted and formed into thin hot film, which is coated onto the moving substrate. The coated substrate then usually passes between a set of counter-rotating rolls, which press the coating onto the substrate to ensure complete contact and adhesion. The alternative is film lamination, where a film of the polymer is supplied and coated onto a heated substrate and pressed onto the substrate by and between a set of counter-rotating rolls to ensure complete contact and adhesion.

The invention will now be explained by means of the following, non-limiting figures.
Figure 1: Schematic process route of starting material for the coating process according to the invention.
Figure 2: Deposition curve as a function of i (A/dm²) for electrolyte solutions with a different chromium(III)concentration (18.1 g/l = 349 mM, 21.2 g/l = 408 mM, 24.9 g/l = 479 mM).
Figure 3: Schematic principle of the chromium deposition mechanism
Figure 4: Chromium coating weight as a function of current density showing the 3 different deposition regimes.

## Claims

1. Method for manufacturing a chromium metal - chromium oxide coated blackplate by electrolytically depositing the chromium metal - chromium oxide coating on blackplate in a continuous high speed plating line operating at a line speed of at least 50 m/min from an electrolyte solution comprising a trivalent chromium compound, wherein the electrolyte solution is free of chloride ions and of a boric acid buffering agent, the electrically conductive substrate acts as a cathode and an anode comprising a catalytic coating of iridium oxide or a mixed metal oxide for reducing or eliminating the oxidation of Cr³⁺-ions to Cr⁶⁺-ions, wherein the electrolyte solution contains at most 250 mM Cr³⁺-ions, a complexing agent at a $\left(\frac{complexing agent}{{Cr}^{3 +}}\right)$ molar ratio of at least 1:1 and at most 2.5:1, wherein the complexing agent is formate (HCOO-), 210 to 2800 mM of sodium sulphate (Na₂SO₄), a pH of between 1.5 and 3.0 measured at 25 °C, and wherein the plating temperature is between 30 and 70 °C.

2. Method according to claim 1 wherein the complexing agent is added to the electrolyte solution as sodium formate (HCOONa).

3. Method according to claim 1 wherein the Cr³⁺-ions are provided by a water soluble chromium(III) salt and wherein the water soluble chromium(III) salt preferably is one or more of the following water soluble chromium(III) salts:
• basic chromium(III)sulphate
• chromium(III)formate
• chromium(III)oxalate
• chromium(III)acetate.

4. Method according to claim 1 or 2 wherein the electrolyte solution contains at most 225 mM of Cr³⁺-ions, and/or at least 100 mM of Cr³⁺-ions, preferably at least 125 mM of Cr³⁺-ions.

5. Method according to any one of the preceding claims wherein the pH of the electrolyte solution is at most 2.8, preferably at most 2.6, more preferably at most 2.2.

6. Method according to any one of the preceding claims wherein the formate/Cr³⁺ molar ratio is at most 2.0:1.

7. Method according to any one of the preceding claims wherein the electrolyte solution contains at least 75 mM and/or at most 600 mM of sodium formate.

8. Method according to any one of the preceding claims wherein the electrolyte solution contains at most 845 mM of sodium sulphate.

9. Method according to any one of the preceding claims wherein the plating temperature is at least 40 °C, preferably at least 50 °C, more preferably at least 55 °C.

10. Method according to any one of the preceding claims wherein the line speed of the plating line is at least 100 m/min.

11. Method according to any one of the preceding claims wherein the coated blackplate is further coated on one or both sides by a film lamination step or a direct extrusion step, with an organic coating consisting of a thermoplastic single layer, or a thermoplastic multi-layer polymer.

12. Method according to claim 11 preferably wherein the thermoplastic polymer coating is a polymer coating system comprising one or more layers comprising thermoplastic resins such as polyesters or polyolefins, acrylic resins, polyamides, polyvinyl chloride, fluorocarbon resins, polycarbonates, styrene type resins, ABS resins, chlorinated polyethers, ionomers, urethane resins and functionalised polymers; and/or copolymers thereof; and or blends thereof.

13. Method according to claim 11 wherein the thermoplastic polymer coating on the one or both sides of the coated blackplate is a multi-layer coating system, said coating system comprising at least an adhesion layer for adhering to the coated blackplate, a surface layer and a bulk layer between the adhesion layer and the surface layer, wherein the layers of the multi-layer coating system comprise or consist of polyesters, such as polyethylene terephthalate, IPA-modified polyethylene terephthalate, CHDM-modified polyethylene terephthalate, polybutylene terephthalate, polyethylene naphthalate, or copolymers or blends thereof.

## Patentansprüche

1. Verfahren zum Herstellen eines mit Chrommetall-Chromoxid beschichteten Schwarzblechs durch elektrolytisches Abscheiden der Chrommetall-Chromoxid-Beschichtung auf Schwarzblech in einer kontinuierlichen Hochgeschwindigkeits-Plattierungslinie, die mit einer Liniengeschwindigkeit von zumindest 50 m/Min. arbeitet, aus einer Elektrolytlösung, umfassend eine dreiwertige Chromverbindung, wobei die Elektrolytlösung frei von Chloridionen und von einem Borsäure-Puffermittel ist, wobei das elektrisch leitfähige Substrat als eine Kathode wirkt und eine Anode umfassend eine katalytische Beschichtung aus Iridiumoxid oder einem gemischten Metalloxid zum Reduzieren oder Eliminieren der Oxidation von Cr³⁺-Ionen zu Cr⁶⁺-Ionen, wobei die Elektrolytlösung höchstens 250 mM Cr³⁺-Ionen enthält, einen Komplexbildner bei einem $\left(\frac{Komplexbildner}{{Cr}^{3 +}}\right)$ Molverhältnis von zumindest 1:1 und höchstens 2,5:1, wobei der Komplexbildner Formiat (HCOO-) ist, 210 bis 2800 mM Natriumsulfat (Na₂SO₄), einen pH zwischen 1,5 und 3,0, gemessen bei 25 °C, und wobei die Plattierungstemperatur zwischen 30 und 70 °C ist.

2. Verfahren nach Anspruch 1, wobei der Komplexbildner der Elektrolytlösung als Natriumformiat (HCOONa) hinzugefügt wird.

3. Verfahren nach Anspruch 1, wobei die Cr³⁺-Ionen durch ein wasserlösliches Chrom(III)-Salz bereitgestellt werden und wobei das wasserlösliche Chrom(III)-Salz bevorzugt eines oder mehrere der folgenden wasserlöslichen Chrom(III)-Salze ist:
• basisches Chrom(III)sulfat
• Chrom(III)formiat
• Chrom(III)oxalat
• Chrom(III)acetat.

4. Verfahren nach Anspruch 1 oder 2, wobei die Elektrolytlösung höchstens 225 mM Cr³⁺-Ionen und/oder zumindest 100 mM Cr³⁺-Ionen, bevorzugt zumindest 125 mM Cr³⁺-Ionen enthält.

5. Verfahren nach einem der vorhergehenden Ansprüche, wobei der pH der Elektrolytlösung höchstens 2,8, bevorzugt höchstens 2,6, bevorzugter höchstens 2,2 ist.

6. Verfahren nach einem der vorhergehenden Ansprüche, wobei das Formiat/Cr³⁺-Molverhältnis höchstens 2,0:1 ist.

7. Verfahren nach einem der vorhergehenden Ansprüche, wobei die Elektrolytlösung zumindest 75 mM und/oder höchstens 600 mM Natriumformiat enthält.

8. Verfahren nach einem der vorhergehenden Ansprüche, wobei die Elektrolytlösung höchstens 845 mM Natriumsulfat enthält.

9. Verfahren nach einem der vorhergehenden Ansprüche, wobei die Plattierungstemperatur zumindest 40 °C, bevorzugt zumindest 50 °C, bevorzugter zumindest 55 °C ist.

10. Verfahren nach einem der vorhergehenden Ansprüche, wobei die Liniengeschwindigkeit der Plattierungslinie zumindest 100 m/Min. ist.

11. Verfahren nach einem der vorhergehenden Ansprüche, wobei das beschichtete Schwarzblech ferner auf einer oder beiden Seiten durch einen Filmlaminierungsschritt oder einen direkten Extrusionsschritt mit einer organischen Beschichtung beschichtet wird, die aus einem thermoplastischen Einzelschicht- oder einem thermoplastischen Mehrschichtpolymer besteht.

12. Verfahren nach Anspruch 11, wobei die thermoplastische Polymerbeschichtung bevorzugt ein Polymerbeschichtungssystem ist, das eine oder mehrere Schichten umfasst, die thermoplastische Harze wie Polyester oder Polyolefine, Acrylharze, Polyamide, Polyvinylchlorid, Fluorkohlenstoffharze, Polycarbonate, Harze vom Styroltyp, ABS-Harze, chlorierte Polyether, Ionomere, Urethanharze und funktionalisierte Polymere; und/oder Copolymere davon; und/oder Mischungen davon umfassen.

13. Verfahren nach Anspruch 11, wobei die thermoplastische Polymerbeschichtung auf einer oder beiden Seiten des beschichteten Schwarzblechs ein mehrschichtiges Beschichtungssystem ist, wobei das Beschichtungssystem zumindest eine Haftschicht zum Anhaften an dem beschichteten Schwarzblech, eine Oberflächenschicht und eine Masseschicht zwischen der Haftschicht und der Oberflächenschicht umfasst, wobei die Schichten des mehrschichtigen Beschichtungssystems Polyester, wie Polyethylenterephthalat, IPA-modifiziertes Polyethylenterephthalat, CHDM-modifiziertes Polyethylenterephthalat, Polybutylenterephthalat, Polyethylennaphthalat, oder Copolymere oder Mischungen davon umfassen oder daraus bestehen.

## Revendications

1. Procédé de fabrication d'une tôle de support revêtue de chrome élémentaire - oxyde de chrome par dépôt électrolytique du revêtement de chrome élémentaire - oxyde de chrome sur la tôle de support dans une chaîne de placage continu à haute vitesse fonctionnant à une vitesse de chaîne d'au moins 50 m/min à partir d'une solution électrolytique comprenant un composé de chrome trivalent, dans lequel la solution électrolytique est exempte d'ions de chlore et d'un agent tampon d'acide borique, le substrat conducteur de l'électricité joue le rôle de cathode et une anode comprenant un revêtement catalytique d'oxyde d'iridium ou d'un oxyde métallique mixte pour réduire ou éliminer l'oxydation des ions Cr³⁺ en ions Cr⁶⁺, dans lequel la solution électrolytique contient au plus 250 mM d'ions Cr³⁺, un agent complexant à un $\left(\frac{agent complexant}{{Cr}^{3 +}}\right)$ rapport molaire d'au moins 1:1 et au plus 2,5:1, où l'agent complexant est un formate (HCOO-), 210 à 2800 mM de sulfate de sodium (Na₂SO₄), un pH compris entre 1,5 et 3,0 mesuré à 25 °C, et où la température de placage est comprise entre 30 et 70 °C.

2. Procédé selon la revendication 1, dans lequel l'agent complexant est ajouté à la solution électrolytique sous forme de formate de sodium (HCOONa).

3. Procédé selon la revendication 1, dans lequel les ions Cr³⁺ sont fournis par un sel de chrome(III) soluble dans l'eau, et dans lequel le sel de chrome(III) soluble dans l'eau est de préférence un ou plusieurs des sels de chrome(III) solubles dans l'eau suivants :
• sulfate de chrome(III) basique
• formate de chrome(III)
• oxalate de chrome(III)
• acétate de chrome(III).

4. Procédé selon la revendication 1 ou 2, dans lequel la solution électrolytique contient au plus 225 mM d'ions Cr³⁺, et/ou au moins 100 mM d'ions Cr³⁺, de préférence au moins 125 mM d'ions Cr³⁺.

5. Procédé selon l'une quelconque des revendications précédentes, dans lequel le pH de la solution électrolytique est au plus 2,8, de préférence au plus 2,6, ou mieux encore au plus 2,2.

6. Procédé selon l'une quelconque des revendications précédentes, dans lequel le rapport molaire formate/Cr³⁺ est au plus 2,0:1.

7. Procédé selon l'une quelconque des revendications précédentes, dans lequel la solution électrolytique contient au moins 75 mM et/ou au plus 600 mM de formate de sodium.

8. Procédé selon l'une quelconque des revendications précédentes, dans lequel la solution électrolytique contient au plus 845 mM de sulfate de sodium.

9. Procédé selon l'une quelconque des revendications précédentes, dans lequel la température de placage est au moins 40 °C, de préférence au moins 50 °C, mieux encore au moins 55 °C.

10. Procédé selon l'une quelconque des revendications précédentes, dans lequel la vitesse de chaîne de la chaîne de placage est au moins 100 m/min.

11. Procédé selon l'une quelconque des revendications précédentes, dans lequel la tôle de support revêtue est en outre revêtue sur un ou les deux côtés, par une étape de lamination par film ou une étape d'extrusion directe, avec un revêtement organique constitué d'une couche thermoplastique simple, ou d'un polymère multicouche thermoplastique.

12. Procédé selon la revendication 11, de préférence dans lequel le revêtement de polymère thermoplastique est un système de revêtement de polymère comprenant une ou plusieurs couches comprenant des résines thermoplastiques telles que polyesters ou polyoléfines, résines acryliques, polyamides, chlorure de polyvinyle, résines d'hydrocarbure fluoré, polycarbonates, résines de type styrène, résines ABS, polyéthers chlorés, ionomères, résines d'uréthane et polymères fonctionnalisés ; et/ou copolymères de ces résines ; et/ou mélanges de ces résines.

13. Procédé selon la revendication 11, dans lequel le revêtement de polymère thermoplastique sur un ou les deux côtés de la tôle de support revêtue est un système de revêtement multicouche, ledit système de revêtement comprenant au moins une couche d'adhésion pour assurer l'adhérence à la tôle de support revêtue, une couche de surface et une couche de volume entre la couche d'adhésion et la couche de surface, dans lequel les couches du système de revêtement multicouche comprennent ou sont constituées de polyesters, tels que polyéthylène téréphtalate, polyéthylène téréphtalate modifié par IPA, polyéthylène téréphtalate modifié par CHDM, polybutylène téréphtalate, polyéthylène naphthalate, ou copolymères ou mélanges de ceux-ci.
